

T. D. MILLER,  
PROTECTED METAL SHEET,  
APPLICATION FILED FEB. 24, 1913.

1,115,714.

Patented Nov. 3, 1914.

Fig. 1.



Fig. 2.



Fig. 3.



Fig. 4.



Fig. 5.



Witnesses:

M. S. Oryer.  
J. Murphy

Inventor,  
Thomas D. Miller  
by Jas. H. Chisholm  
Atty.

# UNITED STATES PATENT OFFICE.

THOMAS D. MILLER, OF CATONSVILLE, MARYLAND, ASSIGNOR TO ASBESTOS PROTECTED METAL COMPANY, OF BEAVER FALLS, PENNSYLVANIA, A CORPORATION OF MASSACHUSETTS.

## PROTECTED METAL SHEET.

1,115,714.

Specification of Letters Patent.

Patented Nov. 3, 1914.

Application filed February 24, 1913. Serial No. 750,105.

*To all whom it may concern:*

Be it known that I, THOMAS D. MILLER, a citizen of the United States, residing in Catonsville, county of Baltimore, and State of Maryland, have invented an Improvement in Protected Metal Sheets, of which the following description, in connection with the accompanying drawings, is a specification, like letters on the drawings representing like parts.

This invention relates to building material of that character in which sheets of asbestos paper or like material are affixed by an asphalt cement to the opposite surfaces 15 of a metal sheet, preferably steel, and substantially such as shown and described in U. S. Patent No. 1,002,303 dated Sept. 5, 1911.

The present invention has for its object to 20 prolong the life and effectiveness of building material of the character described, which is accomplished in accordance with this invention by enveloping the side edges of the asphalt covered metal sheet with 25 folds of asbestos paper, which folds may be secured to or form part of one or both of the asbestos sheets which are affixed to the opposite surfaces of the metal sheet.

Figure 1 is a plan view of one form of 30 building material embodying this invention. Fig. 2, a cross section on the line 2—2, Fig. 1. Figs. 3 and 4 modified forms to be referred to, and Fig. 5, an enlarged section on the line 5—5, Fig. 4.

35 Referring to the drawing *a* represents a metal sheet, preferably steel or iron and which may be of any desired size according to which part of the building it is to be used in, and *b*, *c*, represent sheets or pre-40 formed layers of asbestos paper or the like, which are firmly attached to the metal sheet by an interposed layer *d* of asphalt cement.

The asphalt *d* covers the edges of the metal sheet *a*, and in accordance with the 45 present invention the asphalt which covers the side edges of said metal sheet is enveloped in folds 10, 12, of asbestos paper which extend the length of the metal sheet and which may be secured to or form part 50 of one or both of the sheets *b*, *c*.

In Figs. 1, 2 and 3, the folds 10, 12 are 55 represented as forming part of the asbestos sheet *b*, which in this case is made wider than the metal sheet *a*, so that the opposite sides of the asbestos sheet *b* may be folded

about the side edges of the asphalt covered metal sheet *a* and be carried under and cemented to the asbestos sheet *c*. This construction is advantageous, in that, the sheet *c* may be made of an inferior quality of asbestos paper and the sheet *b* of a superior quality, for in such case, the asbestos protected metal sheet may be placed in the building, so that the inferior asbestos sheet *c* will not be subjected to the same conditions as the asbestos sheet *b*, and consequently need not be of as high grade of asbestos. The asbestos folds 10, 12, envelop the side edges of the metal sheet *a*, and the asphalt *d* which covers the said side edges. 60 As a result, the life and usefulness of the asbestos protected metal sheet as a building material is materially prolonged, for the reason that the asphalt covering the side edges of the metal sheet is itself covered by 65 a thickness of asbestos paper which is opaque and protects the asphalt from the injurious effects of light, air, gases and fumes and also from mechanical abrasion, so that the asphalt is kept from deteriorating and is maintained in its most effective condition for a materially longer time than is the case when the asphalt is exposed to 70 the action of light, air, gases and fumes.

The ends of the metal sheet may be protected by the overlapping ends of the asbestos sheets *b*, *c*, which may be cemented together by the asphalt, as described in the patent referred to, but as these edges are more or less protected in use by having contiguous sheets overlap, the exposure of the asphalt between the asbestos sheets at the 75 ends of the protected metal sheet is not so serious as at the sides of the said sheet.

In Figs. 4 and 5 the folds 10, 12 are 80 formed from a single sheet, which may be the sheet *b* of Fig. 1, which in this case is made wide enough to envelop the sides of the asphalt covered metal sheet *a* and have their ends overlapped, and the overlapping 85 portions of the asbestos sheet may be cemented together with asphalt or other adhesive material. In the present instance the metal sheet *a* is shown as corrugated but it may be flat if desired. So also the protective folds 10, 12 are represented as forming 90 integral parts of one of the asbestos sheets, but they may be separate therefrom and cemented to the sheets *b*, *c*, with asphalt, and also they may form part of both sheets, 95 100 105 110

that is, one fold as 10 may form part of the sheet *b*, and the other fold 12 may form part of the sheet *c*. The protected metal sheet herein shown, may be made of sufficient size 5 to be used in the construction of the roof, side walls or other part of a building or other structure or they may be made of substantially the size of a shingle and used as such in the same manner as the ordinary 10 wooden shingles. In some instances the inferior sheet *c* may be made of paper, felt or like material. The sheet *b* of high grade asbestos is designed to be exposed to the weather and may and preferably will be 15 compacted, hardened and waterproofed, substantially as described in the patent referred to. The ends of the sheets *b*, *c*, may overlap the metal sheet a sufficient amount 20 to enable the said ends to be folded under the ends of the metal sheet, if desired.

Claims.

1. A material of the character described, comprising a metal sheet having affixed to its opposite surfaces by an asphalt cement 25 preformed layers of asbestos and having its side edges covered with asphalt which is enveloped by folds of preformed layers of asbestos extended longitudinally of the metal sheet.
2. A material of the character described, comprising a metal sheet enveloped in a layer of asphalt cement and having affixed to its opposite surfaces preformed sheets 30 of asbestos of different grades, one of the 35 said sheets of asbestos extending from one

surface around both side edges of the metal sheet and overlapping the other sheet of asbestos.

3. A material of the character described, 40 comprising a steel sheet covered with asbestos and having each side edge of the steel sheet inclosed in a continuous fold of asbestos, the said fold being adapted to underlie and overlie the steel sheet, and to be secured thereto by an asphalt cement.

4. A material of the character described, 45 comprising a steel sheet enveloped in a layer of asphalt cement and having fixed to one surface a preformed sheet of asbestos of superior quality and to its other surface an 50 inferior sheet, and folds of asbestos extended longitudinally of the steel sheet and enveloping the opposite side edges of the same, said folds overlying and underlying the metal sheet and being secured thereto by 55 asphalt cement.

5. A material of the character described, comprising a steel sheet covered with asbestos and having each side edge of the 60 steel sheet inclosed in a continuous fold of fibrous material, the said fold being adapted to underlie and overlie the steel sheet, and to be secured thereto by an asphalt cement.

In testimony whereof, I have signed my name to this specification in the presence of 65 two subscribing witnesses.

THOMAS D. MILLER.

Witnesses:

H. H. ROBERTSON,  
F. H. HILL.